

## UNITED STATES PATENT OFFICE

2,404,446

LUBRICANT ADDITIVES AND PREPARATION  
THEREOF

Eugene Lieber, West New Brighton, Staten Island, N. Y., and Aloysius F. Cashman, Bayonne, N. J., assignors to Standard Oil Development Company, a corporation of Delaware

No Drawing. Application December 30, 1942,  
Serial No. 470,642

1 Claim. (Cl. 260—125)

1

This invention relates to improved extreme pressure additives for incorporation in mineral lubricating oils to prepare lubricants especially adapted for operation under extreme pressure, such as involved in the operation of hypoid gears used in motor vehicles, etc.

It has been known for some time that mineral oils per se are not capable of withstanding the great pressures encountered between engaged metal surfaces in various types of machines, etc., such as hypoid gears, but that additives capable of increasing their load carrying capacity to a satisfactory degree can be made by making petroleum hydrocarbon derivatives containing both sulfur and a halogen such as chlorine. Such additives may be made, for instance, as described in U. S. Patent 2,124,598, by chlorinating a petroleum hydrocarbon fraction such as kerosene or paraffin wax and reacting the resultant chlorinated hydrocarbon product with alkaline polysulfide. Other related products are made by reacting a chlorinated kerosene with alkaline xanthates, alkaline-thiocyanates, alkaline mercaptides, etc. Although such extreme pressure additives have in general been quite satisfactory, it has been observed occasionally that some of these additives have shown a slight tendency toward instability during storage, apparently due to the presence therein of constituents which either are not as completely soluble or tend to become insoluble and settle out during storage.

It is one object of the present invention to prepare extreme pressure additives which are substantially free from any constituents which are either insoluble or tend to become insoluble during storage. Another object of the invention is to improve the load carrying capacity of extreme pressure additives.

Broadly the invention comprises refining petroleum hydrocarbon derivatives which contain both sulfur and halogen by contacting them with a selective solvent having a preferential solvency for relatively low-sulfur constituents as compared to relatively high-sulfur constituents.

The invention may be carried out in a number of different ways such as by contacting the original extreme pressure additive, i. e., the crude petroleum hydrocarbon derivative fraction containing both sulfur and halogen, with a selective solvent, preferably with suitable agitation,

and then allowing the mixture to settle into two layers, one the extract phase (usually the upper layer) and the other the raffinate phase (usually the lower layer). Such a batch extraction may be repeated successively until the desired separation has been made by the desired constituents having good stability and good extreme pressure lubricating characteristics, which generally are constituents having about 1 to 10% of sulfur and about 30 to 40% of chlorine, as distinguished from the undesirable fraction which generally has such poor stability as to be actually insoluble in mineral lubricating oils and which generally has more than 10% of sulfur and less than 30% of chlorine. This type of extraction may be illustrated by the use of isopropyl alcohol as the extracting solvent, in which case the desired constituents are dissolved preferentially in the solvent and therefore are contained in the extract phase while the undesired constituents remain in the raffinate phase.

Such solvent extraction may be carried out either by batch operation using one or a plurality of successive batches or stages, using either fresh or recycled solvent, or it may be carried out continuously; and it may also be carried out concurrently or countercurrently. A preferred procedure is continuous countercurrent solvent extraction, illustrated by feeding a solvent such as isopropyl alcohol into the base of a vertical tower and feeding the original or crude extreme pressure additive (which has a higher gravity than the alcohol) near the top thereof so that it will descend while the alcohol is ascending with the result that a countercurrent contacting is carried out continuously, the alcohol extract phase being removed continuously from the top of the tower and the undesired insoluble raffinate being removed continuously at the bottom of the tower.

Another way of carrying out the invention is to mix the crude extreme pressure additive with a suitable solvent, heat to the point of complete solubility or miscibility, and then either cool and/or add a precipitating agent or anti-solvent to cause the separation into two liquid phases.

The material to be used as solvent may be selected from a wide variety of substances. Examples include the lower alcohols such as isopropyl alcohol, amyl alcohol, butyl alcohol, ethyl alcohol, etc., or various other types of oxygen

containing aliphatic organic compounds, such as ethers, e. g., di-ethyl ether, di-isopropyl ether, etc., ketones, e. g., acetone, methyl isopropyl ketone, methyl isobutyl ketone, etc., esters, e. g., ethyl acetate, isopropyl acetate, amyl acetate, methyl propionate, isopropyl butyrate, ethyl valerate, etc., or organic acids, such as acetic acid, chloracetic acid, propionic acid, etc. Other substances known more or less as a class of selective solvents having a preferential solvency for aromatic and unsaturated hydrocarbons may be used such as phenol, liquid sulfur dioxide, aniline, furfural, dichlor diethyl ether, nitrobenzene, etc. A still different type of solvent which may be used comprises liquefied normally gaseous hydrocarbons such as butane, propane, ethane, etc.

In carrying out the solvent extraction with any of the various types of solvents mentioned above, instead of using a single solvent, two or more different solvents either within the same class of substances or in different classes may be used. Also, if desired, various substances, known as anti-solvents in the lubricating oil solvent extraction art, may be used such as water, glycols, liquid anhydrous ammonia, etc.; such materials are preferably used in relatively small amounts to modify the solvency characteristics of one of the other types of solvents mentioned above. A still further alternative procedure is to dilute the crude extreme pressure additive with a light hydrocarbon liquid, such as a refined naphtha, before contacting it with the selective solvent.

After the extraction has been completed, the solvent may be removed from the solvent phase and this may be done either after individual steps in a process involving several stages, or at the end of a cumulative or countercurrent operation.

In carrying out the invention the proportions of materials to be used will, of course, vary within a wide range depending upon the nature of the crude extreme pressure additive being treated, the type of solvent, and anti-solvent (if any) used, as well as upon the temperature and pressure conditions used and the degree of refinement desired. However, usually about  $\frac{1}{2}$  to 10 parts of solvent should be used to one part by volume of crude extreme pressure additive, and generally about 1 to 5 volumes of solvent to one of extreme pressure additive will be found to give satisfactory results. The temperature used may be either room temperature or above or below room temperature, and generally a temperature between room temperature and  $250^{\circ}$  F. will be satisfactory. The pressure may be atmospheric or above or below atmospheric, a slight superatmospheric pressure being, of course, necessary when using volatile materials, such as liquefied normally gaseous hydrocarbons.

The objects, advantages and details of the invention will be better understood from a consideration of the following specific examples which are offered by way of illustration but without the intention of limiting the invention specifically thereto.

#### EXAMPLE 1

A sample of commercial extreme pressure additive marketed under the trade name "Parapoid-10," made by chlorinating kerosene at a temperature of about  $175^{\circ}$  F. to a chlorine content of about 40% chlorine, and reacting the resulting chlorinated kerosene with sodium polysulfide, and also found to contain 7.3% sulfur and 33.0% chlorine, was used as raw material according to this invention. About 1,200 grams of this mate-

rial, referred to as crude extreme pressure agent A, was contacted very vigorously with 1,000 cc. of isopropyl alcohol (91% grade) in a separatory funnel and the mixture settled at room temperature for 48 hours. The following separation was effected.

Extract phase (upper layer) = 1,040 cc.  
Raffinate phase (lower layer) = 960 cc.

The extract phase was distilled in order to remove the isopropyl alcohol, taking off the last traces under high vacuum on a water bath. An extract weighing 112 grams was obtained. This will be identified as "First extraction" product.

The raffinate phase obtained above was contacted very vigorously with 1,000 cc. of 99% isopropyl alcohol by contacting vigorously in a separatory funnel and the mixture settled for 24 hours at room temperature. The following separation was effected:

Second extract phase (upper layer) = 1,240 cc.  
Second raffinate phase (lower layer) = 710 cc.

The second extract phase was distilled as before and a "Second extraction" product weighing 363 grams was obtained.

The "Second raffinate" phase was contacted vigorously again with 1,000 cc. of 99% isopropyl alcohol as before. After settling for 72 hours at room temperature the following separations were obtained:

Third extract phase (upper layer) = 1,220 cc.  
Third raffinate phase (lower layer) = 500 cc.

The third extract phase was distilled as before to remove isopropyl alcohol and a "Third extraction" product weighing 201 grams was obtained.

The "Third raffinate" phase obtained above was contacted vigorously again with 1,000 cc. of 99% isopropyl alcohol. After settling for 24 hours the following separation was obtained.

Fourth extract phase (upper layer) = 1,120 cc.  
Fourth raffinate phase (lower layer) = 360 cc.

The fourth extract phase was distilled as before to remove isopropyl alcohol and a "Fourth extraction" product weighing 134 grams was obtained.

The fourth raffinate phase which was becoming quite viscous was given a final extraction with 1,500 cc. of 99% isopropyl alcohol as before. The contacting was carried out at  $125^{\circ}$  F. in order to aid handling because of the high viscosity of the raffinate phase at this point. After settling for 8 days at room temperature, the following separation was obtained:

Fifth extract phase (upper layer) = 1,600 cc.  
Fifth raffinate phase (lower layer) = 260 cc.

The fifth raffinate phase was found to be extremely viscous.

The fifth extract phase was distilled as before to remove isopropyl alcohol and a "Fifth extraction" product weighing 99 grams was obtained. The fifth raffinate phase was also subjected to distillation and a "final" raffinate product weighing 313 grams and consisting of an extremely viscous tar-like material was obtained.

The extract products and the final raffinate product were tested for the following points:

Solubility at 10% concentration in Panhandle Bright Stock Analysis for sulfur and chlorine  
Extreme pressure properties as measured by the SAE machine

The data obtained are summarized in Table 1.

TABLE 1  
Solvent extraction of Parapoid-10  
EXAMPLE NO. 1

| Fraction                                      | Per cent yield <sup>1</sup> | Analysis  |            | Solubility characteristics |                              | Extreme pressure properties <sup>2</sup><br>SAE No. <sup>3</sup> |
|-----------------------------------------------|-----------------------------|-----------|------------|----------------------------|------------------------------|------------------------------------------------------------------|
|                                               |                             | Percent S | Percent Cl | 5% blend in Varsol         | 10% blend in Panhandle B. S. |                                                                  |
| Original unextracted extreme pressure agent A |                             | 7.3       | 33.0       | Cloud and sediment         | Cloud and sediment           | 320                                                              |
| First extraction product                      | 9.4                         | 1.9       | 35.0       | Clear                      | Clear                        | 400                                                              |
| Second extraction product                     | 23.6                        | 3.2       | 35.7       | do                         | do                           | 363                                                              |
| Third extraction product                      | 16.8                        | 3.4       | 33.0       | do                         | do                           | 425                                                              |
| Fourth extraction product                     | 11.2                        | 3.3       | 36.0       | do                         | do                           | 390                                                              |
| Fifth extraction product                      | 8.3                         | 5.6       | 35.5       | do                         | do                           | 398                                                              |
| Raffinate                                     | 26.2                        | 17.0      | 24.4       | Heavy tarry sediment       | Heavy tarry sediment         | -----                                                            |

<sup>1</sup> These are weight yields based on the original unextracted Parapoid-10.<sup>2</sup> 10% blend of particular fraction in Panhandle Bright Stock.<sup>3</sup> This test is described in the S. A. E. Journal, volume 39, pages 23 to 24 for the year 1936.

It will be noted that all of the extracted phases have excellent solubility in both Varsol and Panhandle Bright Stock as contrasted with the original unextracted extreme pressure agent A. "Varsol" is a refined varnolene in the heavy naphtha boiling range. The data also bring out the hitherto unknown fact that materials of the Parapoid type containing only relatively small quantities of sulfur have even better extreme pressure properties, as measured by the S. A. E. testing machine, than the original unextracted material. It was hitherto believed that in order to function as an extreme pressure additive the material had to have a relatively high percentage of sulfur in the molecule.

It is believed that the improvements in solubility characteristics are due essentially to the removal of the heavy tarry material comprising the "raffinate." It was found that this material immediately precipitated not only from Varsol and Panhandle Bright Stock but also from less highly refined petroleum oil fractions.

## EXAMPLE 2

742 grams of commercial Parapoid, referred to as crude extreme pressure agent B, having the following analysis:

% S=6.4

% Cl=32.3

was subjected to solvent fractionation by the procedure of Example 1, except that 99% isopropyl alcohol was used as solvent throughout.

The data obtained are summarized in Table 2.

TABLE 2  
Solvent extraction of Parapoid-10  
EXAMPLE NO. 2

| Fraction                      | Percent yield <sup>1</sup> | Analysis  |            | Solubility characteristics 10% blend in Panhandle B. S. | Extreme pressure properties <sup>2</sup><br>S. A. E. number <sup>3</sup> |
|-------------------------------|----------------------------|-----------|------------|---------------------------------------------------------|--------------------------------------------------------------------------|
|                               |                            | Percent S | Percent Cl |                                                         |                                                                          |
| Original unextracted material |                            | 6.4       | 32.3       | Clear                                                   | 290                                                                      |
| First extraction product      | 11.8                       | 1.8       | 34.2       | Cloud (slight)                                          | 372                                                                      |
| Second extraction product     | 35.9                       | 4.1       | 33.8       | Clear                                                   | 388                                                                      |
| Third extraction product      | 19.6                       | 4.1       | 34.6       | do                                                      | 443                                                                      |
| Fourth extraction product     | 7.6                        | 5.0       | 34.3       | do                                                      | 418                                                                      |
| Raffinate                     | 19.7                       | 16.0      | 25.0       | Precipitates out as a tar                               | -----                                                                    |

<sup>1</sup> These are weight yields based on the original unextracted Parapoid-10.<sup>2</sup> 10% blend of the particular fraction in Panhandle Bright Stock.<sup>3</sup> This test is described in the S. A. E. Journal, volume 39, pages 23 to 24, for the year 1936.

## EXAMPLE 3

600 gms. of Parapoid-10, containing 6.5% S and 32% Cl, were placed in a tall vertical glass cylinder used as extractor and 1500 cc. of 98% 75

As indicated above, even in this small-scale laboratory continuous extraction, the extract was remarkably superior to the original crude extreme pressure agent in regard to solubility and stability, while the raffinate developed a heavy cloud

and sediment in the solubility test and showed excessive copper corrosion.

This type of continuous extraction can be carried out on a commercial scale by using a large vertical tower extractor, which may contain packing material or baffle plates, if desired, in

were subjected to solvent fractionation by the procedure of Example 1, except that 91% isopropyl alcohol was used as solvent in the first three extractions and 99% isopropyl alcohol in the fourth and fifth. The data is summarized below.

TABLE  
Solvent extraction of Santapoid-A

| Fraction               | Percent yield <sup>1</sup> | Analysis  |            | Solubility characteristics 10% blend in Panhandle Bright Stock <sup>2</sup> | Extreme pressure properties S. A. E. No. |
|------------------------|----------------------------|-----------|------------|-----------------------------------------------------------------------------|------------------------------------------|
|                        |                            | Percent S | Percent Cl |                                                                             |                                          |
| Santapoid-A            |                            | 9.6       | 31.6       | Cloud and slight sediment.                                                  | 340                                      |
| 1st extraction product | 16.6                       | 6.7       | 33.4       | Clear and no sediment.                                                      | 380                                      |
| 2nd extraction product | 20.4                       | 6.9       | 35.2       | do                                                                          | 365                                      |
| 3rd extraction product | 16.0                       | 7.8       | 34.8       | do                                                                          | 365                                      |
| 4th extraction product | 42.3                       | 10.5      | 32.8       | do                                                                          | 365                                      |
| 5th extraction product | 9.0                        | 11.9      | 31.9       | do                                                                          | 405                                      |
| Raffinate              | 9.0                        | 23.8      | 20.8       | Heavy tarry sediment                                                        | 280                                      |

<sup>1</sup> These are weight yields based on original unextracted Santapoid.

<sup>2</sup> 10% by weight of the particular fraction in Panhandle Bright Stock.

order to obtain better contacting of the up-going and down-going liquids, then feeding the crude extreme pressure agent into the tower near the top thereof and feeding the alcohol in near the bottom of the tower, continuously withdrawing the solvent extract phase at the top and the raffinate at the bottom of the tower, continuously passing the solvent extract phase to a reboiler or still from which the alcohol is continuously vaporized and from which the solvent free extract is withdrawn, the alcohol vapors being continuously condensed and recycled to the extraction tower.

#### EXAMPLE 4

A commercial extreme pressure agent known as Santapoid A (previously referred to above) is said to be prepared as follows:

Isopropyl alcohol is heated with anhydrous sodium hydroxide and then carbon disulfide is added to form isopropyl xanthate.



Chlorinated kerosene is then added in the proper proportion and the mixture is refluxed. Sodium chloride splits out and the Santapoid is formed.



585 gms. of this commercial Santapoid-A having the following analysis:



It is thus seen that by means of the present invention it is possible to make extreme pressure additives which have a much better temperature and storage stability, especially in the presence of metals, and also such products having superior extreme pressure lubricating characteristics, as compared to the original or crude extreme pressure additives.

It is not intended that this invention be limited to the specific examples which have been given merely for the sake of illustration but only by the appended claim in which it is intended to claim all novelty inherent in the invention as well as all modifications coming within the scope and spirit of the invention.

We claim:

Process of preparing improved extreme pressure lubricating agents which comprises solvent extracting a chlorinated paraffin alkali polysulfide reaction product containing about 5 to 10% of sulphur and about 30 to 40% of chlorine at about room temperature with isopropyl alcohol of about 91% concentration, using about 1000 cc. of the alcohol per 1200 grams of material treated, separating the raffinate phase from the extract phase, subjecting the raffinate phase to three successive extractions at room temperature with isopropyl alcohol of about 99% concentration, using about the same volume of solvent as in the first extraction phase, extracting the fourth raffinate at about 125° F. with isopropyl alcohol of about 99% concentration, and recovering the solvent from each of the extract phases and from the final raffinate phase.

EUGENE LIEBER.

ALOYSIUS F. CASHMAN.